

## 1

3,698,969

### SOLID STABILIZED HYDRAZINIUM DIPERCHLORATE PROPELLANT

Marvin Fein, Westfield, Frank Loprest, Chester, and  
Donald G. Shaheen, Dover, N.J., assignors to Thiokol  
Chemical Corporation, Bristol, Pa.  
No Drawing. Filed Sept. 10, 1965, Ser. No. 486,552  
Int. Cl. C06d 5/06

U.S. Cl. 149—19

17 Claims

#### ABSTRACT OF THE DISCLOSURE

A solid propellant having hydrazinium diperchlorate as the oxidizer in a hydrocarbon fuel binder contains a stabilizing amount of a chelating agent for stabilization with respect to vibrational and thermal shock. Also included are various propellant adjuvants for additional performing characteristics.

This invention concerns stabilized oxidizer compositions and their preparation.

More particularly, this invention relates to the preparation of stabilized hydrazinium diperchlorate oxidizer composition using small quantities of metal chelating agents as the stabilizing agents.

Hydrazinium diperchlorate (HP<sub>2</sub>) is an exceeding energetic oxidizer. In addition to its potency, it has certain other advantages which would make it a desirable oxidizer component in solid propellant compositions. These advantages include high density and a high burning rate. In addition, the composition is available in large quantities in a high state of purity at relatively moderate cost. The high density of HP<sub>2</sub> permits high loading levels compared to many less energetic oxidizers. This in turn increases the available energy of the propellant composition on a unit weight basis and increases the potential range of the rocket hardware. All of these attributes of HP<sub>2</sub> are important considerations in military and aerospace operations.

Unfortunately, HP<sub>2</sub> has an important defect which has curtailed its widespread use. This shortcoming is its relatively poor stability to vibrational and thermal shock especially when formulated with the usual polymeric fuel binder and propellant adjuvants. While the oxidizer can be prepared by a number of processes, including neutralization and metatheses, the HP<sub>2</sub> product obtained is sensitive to thermal or mechanical shock, i.e., shock can induce its decomposition, which can proceed either as a deflagration or a detonation.

Because of its poor shock sensitivity, in the present state of the art, extreme care must be used in the storage, handling, and formulation of HP<sub>2</sub>-based propellants. In fact the poor sensitivity of HP<sub>2</sub> presently limits the size of the batches of HP<sub>2</sub> based propellant and presently restricts its use solely to experimental purposes.

In view of the potential value of HP<sub>2</sub> as a propellant oxidizer and because of its relatively high sensitivity, a need exists for a method of preparing HP<sub>2</sub> compositions stable toward mechanical and thermal shock. A desirable method would decrease the mechanical and thermal sensitivity of HP<sub>2</sub> severalfold, would utilize readily available and inexpensive stabilizers and could be utilized by relatively unskilled personnel without the need for special

## 2

equipment. Ideally the stabilizer could be used in sufficiently small quantities so that the potential energy of the oxidizer would not be appreciably diminished. A stabilizing process possessing these advantages would represent a substantial advance in the propellant art.

It is therefore an object of this invention to prepare hydrazinium diperchlorate compositions having improved stability to detonation by vibrational and thermal shock.

It is a further object of this invention to develop a process for preparing the above compositions inexpensively, from readily available materials without the need for special techniques or equipment.

Yet a further object of this invention is the preparation of HP<sub>2</sub> based propellant compositions stabilized toward mechanical and vibrational shock.

Additional objects will become apparent to the reader after a perusal of this application.

In practice, a stabilizing quantity of a stabilizing agent is contacted with HP<sub>2</sub> product or its aqueous or non-aqueous solutions until a homogenous stabilized HP<sub>2</sub> composition is produced.

In the preferred practice, about 0.1 to 10% by weight of ethylene-diaminetetraacetic acid (EDTA) is added to a reaction mixture containing HP<sub>2</sub>, prior to the final crystallization which precedes the final drying step.

The term stabilizing agent as used throughout this application refers to that quantity of stabilizer required to substantially improve the sensitivity of HP<sub>2</sub> to detonation by thermal or vibrational shock. The quantity of stabilizer required varies according to the particular stabilizer used. However in most instances the amount of stabilizer required varies between 0.01 to 10.0% by weight of the HP<sub>2</sub> treated.

The stabilizers of this invention are of diverse origin and structure. For this reason they cannot be described structurally. However, interestingly enough, all of the stabilizers appear to have the ability to form soluble complexes with metallic ions and are referred to in the art as chelating agents. In addition to the preferred ethylenediaminetetraacetic acid and its salts, the following chelating agents can be used: polycarboxylic acids such as malonic acid, ethylmalonic acid, nitrilotriacetic acid, amines such as ethylenediamine, N,N-dimethylmethylenediamine, diethylenetriamine, 1,2,3 - triaminopropane, bi-pyridyl, amino acids and peptides such as alanine, glycine, aspargine, methionine, valine, aminoethylphosphonic acid, ethylenediamine N,N - diacetic acid, ethylenediaminetetrapropionic acid, hydroxy acids such as salicylic acid, sulfosalicylic acid, hydroxy aldehydes such as salicylaldehyde and its alkoxy, halo and alkyl derivatives, B ketones such as benzoylacetone, acetylacetone, thenoyltrifluoroacetone, phenolics such as 8 - hydroxyquinoline, 3,5-difluoropyrocatechol among many others.

To set forth the advantages and working of this invention in the greatest possible detail the following illustrative embodiments are submitted.

In one embodiment, a sample of hydrazinium diperchlorate in a 70% by weight perchloric acid mother liquor (produced in a neutralization of aqueous hydrazine with concentrated (72% by weight) perchloric acid), is divided into two equal portions. To one stirred portion is added 8% by weight (of the HP<sub>2</sub>) of ethylenediaminetetraacetic acid. After 15 minutes of stirring, the treated solution is cooled to -10° C. and the precipitated hydrazinium diperchlorate filtered off. After drying under

vacuum for 15 hours a propellant grade HP<sub>2</sub> product is obtained.

The second portion of the hydrazinium diperchlorate in perchloric acid is processed as above except that no treatment with ethylene diamine tetraacetate acid is given before cooling, precipitation and vacuum drying of the final product.

The treated product and untreated product separately are each admixed with separate portions of CP grade iron powder amounting to 1.3% of its weight and heated to 120° C. in a sealed Pyrex glass tube. After 11 minutes the untreated sample of product decomposes. The EDTA treated sample decomposes after about 53 minutes. This approximately 5 fold decrease in thermal stability is both significant and unexpected. A large decrease in sensitivity toward shock between the two samples is also observed.

In another embodiment, the anhydrous HP<sub>2</sub> derived from a metathetical preparation is divided into two parts. The first part is treated with 8% its weight of EDTA and vacuum dried. The second part is untreated and dried under the same vacuum conditions. Again each portion is treated with about 2% its weight of CP 100 mesh iron powder. Both samples are heated to 125° C. The same order of decreased sensitivity toward thermal shock is observed.

In a further embodiment a 15 parts by weight sample of CP anhydrous, hydrazinium diperchlorate in 100 parts by weight of 72% by weight perchloric acid is treated with 1.5 parts by weight of nitrilotriacetic acid. The mixture is stirred for 15 minutes cooled to -10° C. and filtered. The filter cake is dried for 6 hours under 5 mm./Hg. A substantial decrease in sensitivity toward detonation from vibration and thermal shock is noted compared to untreated control material.

In a further embodiment a 15 parts by weight sample of CP anhydrous, hydrazinium diperchlorate in 100 parts by weight of 72% by weight perchloric acid is treated with 1.5 parts by weight of methionine. The mixture is stirred for 15 minutes cooled to -10° C. and filtered. The filter cake is dried for 16 hours under 5 mm./Hg. A substantial decrease in sensitivity toward detonation from vibration and thermal shock is noted compared to untreated control material.

In a further embodiment a 15 parts by weight sample of CP anhydrous, hydrazinium diperchlorate in 100 parts by weight of 72% by weight perchloric acid is treated with 1.5 parts by weight of ethylenediaminetetrapropionic acid. The mixture is stirred for 15 minutes cooled to -10° C. and filtered. The filter cake is dried for 18 hours under 5 mm./Hg. A substantial decrease in sensitivity toward detonation from vibration and thermal shock is noted compared to untreated control material.

In a further embodiment a 15 parts by weight sample of CP anhydrous, hydrazinium diperchlorate in 100 parts by weight of 72% by weight perchloric acid is treated with 1.5 parts by weight of 8-hydroxyquinoline. The mixture is stirred for 15 minutes cooled to -10° C. and filtered. The filter cake is dried for 6 hours under 5 mm./Hg. A substantial decrease in sensitivity toward detonation from vibration and thermal shock is noted compared to untreated control material.

In a further embodiment a 15 parts by weight sample of CP anhydrous, hydrazinium diperchlorate in 100 parts by weight of 72% by weight perchloric acid is treated with 1.5 parts by weight of sodium tripolyphosphate. The mixture is stirred for 15 minutes cooled to -10° C. and filtered. The filter cake is dried for 14 hours under 5 mm./Hg. A substantial decrease in sensitivity toward detonation from vibration and thermal shock is noted compared to untreated control material.

In a further embodiment a 15 parts by weight sample of CP anhydrous, hydrazinium diperchlorate in 100 parts by weight of 72% by weight perchloric acid is treated with 1.5 parts by weight of salicylic acid. The mixture is stirred for 15 minutes cooled to -10° C. and filtered. The filter

cake is dried for 16 hours under 5 mm./Hg. A substantial decrease in sensitivity toward detonation from vibration and thermal shock is noted compared to untreated control material.

5 In further embodiments, a substantial decrease in sensitivity toward detonation from thermal shock is observed when 5 parts by weight samples of CP grade anhydrous hydrazinium diperchlorate are treated with 0.5 part by weight of the following chelating agents and vacuum dried.

10 CHELATING AGENTS APPLIED

|              |                         |
|--------------|-------------------------|
| Malonic acid | Sulfosalicylic acid     |
| Glycine      | Benzoylacetone          |
| Asparagine   | Thenoyltrifluoroacetone |
| Valine       | 3,5-disulfopyrocatechol |

15 The stabilized hydrazinium diperchlorate of this invention can be formulated with the usual propellant components to form the finished propellant composition. The components include in addition to the stabilized HP<sub>2</sub> of this invention, the components shown below in the proportions indicated.

(1) 10 to 40 parts by weight of a combustible fuel binder,  
(2) 0 to 25 parts by weight of propellant adjuvants.

20 25 The components are admixed until a homogenous mixture is produced then loaded into a rocket motor for curing to the desired physical state. A description of these propellant components is given below.

Binders

30 The binders that can be used with the stabilized HP<sub>2</sub> of this invention are saturated and unsaturated hydrocarbon polymers. A favored group are the polyalkyldienes containing reactive sites such as hydroxy, carboxy, carbonyl, epoxy, amino, imino, and the like. Most of these polymers are commercially available products or can be made using known polymerization procedures. For example, polyalkadienes containing carboxyl groups can be prepared by polymerizing or reacting many materials including conjugated dienes containing from 4 to 8 carbon atoms. These include 1,3-butadiene, isoprene, piperylene, methylpentadiene, 2-ethyl-1,3-butadiene, phenylbutadiene, 3,4-dimethyl-1,3-hexadiene, 4,5-diethyl-1,3-octadiene among others. In addition, conjugated dienes containing reactive substituents along the chain can also be employed, such as for example, halogenated dienes, such as chloroprene, fluoroprene, etc. Of the conjugated dienes, the preferred material is butadiene, with isoprene and piperylene also being especially suitable. In addition to the conjugated dienes, other monomers which can be employed are aryl-substituted olefins, such as styrene, various alkyl styrenes, para-methoxystyrene, vinylnaphthalene, vinyltoluene, and the like; heterocyclic nitrogen containing monomers, such as pyridine and quinoline derivatives containing at least 1 vinyl or alphamethylvinyl group, such as 2-vinylpyridine, 3-vinylpyridine, 4-vinylpyridine, 3-ethyl-5-vinylpyridine, 2-methyl-5-vinylpyridine, 3,5-diethyl-4-vinylpyridine, etc. In addition, mono- and di- substituted alkenyl pyridines and the like quinolines; acrylic acid esters, such as methyl acrylate, ethyl acrylate; alkacrylic acid esters, such as methyl methacrylate, ethyl methacrylate, propyl methacrylate, butyl methacrylate, methyl vinyl ether, vinyl chloride, vinylidene chloride, vinylfuran, vinylcarbazole, vinylacetylene, etc., can be used as polymer substrates.

40 45 50 55 60 65 70 75 The above compounds, in addition to being polymerizable alone, are also copolymerizable with each other and may be copolymerized to form terminally reactive polymers. In addition, copolymers can be prepared, using minor amounts of copolymerizable monomers containing more than one vinylidene group such as 2,4-divinylpyridine, divinylbenzene, 2,3-divinylpyridine, 3,5-divinylpyridine, 3,5-divinylpyridine, 2,4-divinyl-6-methylpyridine, 2,3-divinyl-5-ethylpyridine, and the like.

Another group of superior binders are the saturated binders containing free carboxyl sites. These binders,

which are the condensates of saturated glycols and saturated acids, are advantageous in certain respects compared to the corresponding polyalkadiene binders. For example, they are more energetic on a weight basis and they are more compatible with HP<sub>2</sub> because they do not contain unsaturated carbon to carbon bonds. A specific saturated binder which is favored is the condensate of neopentyl glycol and Emery 3389 (a proprietary dimer acid condensation polymer sold by Emery Industries); also favored are the halogenated saturated binders such as the carboxyl containing flouroalkanes, and carboxyl terminated alkane polymers such as carboxyl terminated polyisoprene.

The polymeric fuel binders of this invention can range in molecular weight from 250-12,000 or more, although the most satisfactory results have been obtained using carboxyl terminated hydrocarbon polymers ranging in molecular weight between 500-6,000. As indicated, especially favored are the carboxyl terminated polybutadienes and the neopentyl glycol condensate of that molecular weight range.

#### Propellant adjuvants

In addition to the curing agents, accelerators, polymerization and vulcanization catalysts and the like which are included within the fuel binder content of the inventive propellant compositions, certain additives, ignition catalysts, conditioning or modifying agents, surfactants, high energy metals, their hydrides and the like can often be advantageously added to the propellant compositions to alter or improve their physical and combustion characteristics. For convenience sake, these substances are herein generically referred to as propellant adjuvants and they can be present in the finished propellant composition in amounts up to about 30 parts by weight down to 0 part by weight of the final propellant composition.

More commonly, however, the adjuvants comprise from about 20 parts by weight or even less down to about 5 parts by weight of propellant compositions. Among the many propellant adjuvants which can be used are included the following typical materials. Plasticizers such as the alkyl-phthalates and the like, darkening agents such as carbon black or lamp black, ballistic agents such as potassium sulfate, hygroscopicity inhibitors, such as dinitro-toluene and various coolants, combustion and burning rate catalysts. The combustion catalysts are of diverse structure but generally are compounds containing oxygen. These catalysts can be inorganic or organic compounds. They include, among many others, such as ferrous, ferric, magnesium, titanium, calcium, molybdenum, and vanadium oxides and the like. Especially effective as combustion catalysts are the chromates and dichromates, generally with ammonium dichromate being a preferred catalyst. Organics such as nitrocellulose can also be effectively used.

A favored group of adjuvants are the finely divided lightweight and high energy metals and nonmetals such as aluminum, beryllium, boron, silicon and the like. These materials can be used by themselves, as their carbides and hydrides, or they can be employed in the form of their polymer coated particles.

To demonstrate the preparation of typical HP<sub>2</sub> based propellants stabilized toward vibrational and thermal shock the following embodiments is submitted.

In one illustrative embodiment of this invention, the following propellant components are blended in an appropriately sized mixing vessel equipped with an efficient means of blending, cooling and heating in the manner described.

To a stirred 13 parts by weight portion of commercially available carboxy terminated polybutadiene having a molecular weight range between 500 and 6000. (Thiokol HC polymer) is added to 2 parts by weight of 1,1'-ethylenbis(2-ethyl)aziridine curing agent and 16 parts by weight degreased aluminum powder (having a particle size between 3 and 30 microns). After the mixture appears to be uniform, a 70 parts by weight portion of stabilized an-

hydrous propellant grade hydrazinium diperchlorate previously treated by 10% its weight of ethylenediaminetetraacetic acid is blended in. The blending and mixing operation is continued for an additional 30-90 minutes and is cast into a 1/2 lb. rocket engine casing. The propellant is cured at 135° F. for 96 hours. The cured propellant had good flexibility and Shore A hardness.

As indicated earlier this invention is advantageous in both its process and composition aspects.

In its process aspects this invention permits the stabilization of HP<sub>2</sub> toward thermal and vibrational shock by the incorporation of a small quantity of an inexpensive stabilizer to the HP<sub>2</sub> prior to use. No special application equipment or techniques are required and the source of the HP<sub>2</sub> is not important to success.

In its compositional aspects, this invention permits the use of highly energetic propellant compositions than has previously been possible. Further, these compositions withstand handling and storage under operational conditions with less hazard than was heretofore thought possible.

As the above discussions and previous embodiments have indicated numerous modifications and changes in this invention are possible without departing from the inventive concept. The metes and bounds of this invention are best indicated by the claims which follow.

What is claimed is:

1. A hydrazinium diperchlorate composition capable of curing to a solid and stabilized toward vibrational and thermal shock consisting essentially of from .85 to 8.5 parts by weight of a metal chelating agent selected from the group consisting of:

Alkylenediamines

Alkylenetriamines

35 Polycarboxylic acids

Nitrolotriacetic acid

Amino acids

Peptides

The acids and salts of alkylenediamines and alkylene-40 triamines

Hydroxy acids

Hydroxy aldehydes

β-ketones

45 Phenolics, from about 10 to 40 parts by weight of a combustible polymeric hydrocarbon fuel binder including a curing agent in admixture therewith, and from about 45 to 85 parts by weight of hydrazinium diperchlorate.

2. The composition of claim 1 wherein the stabilizing agent is ethylenediaminetetraacetic acid.

50 3. The composition of claim 1 wherein the stabilizing agent is nitrolotriacetic acid.

4. The composition of claim 1 wherein the stabilizing agent is methionine.

55 5. The composition of claim 1 wherein the stabilizing agent is ethylenediaminetetrapropionic acid.

6. The composition of claim 1 wherein the stabilizing agent is 8-hydroxyquinoline.

7. The composition of claim 1 wherein the stabilizing agent is sodium tripolyphosphate.

60 8. The composition of claim 1 wherein the stabilizing agent is salicylic acid.

9. The composition of claim 1 wherein the stabilizing agent is benzoylacetone.

65 10. The composition of claim 1 wherein the stabilizing agent is thenoyltrifluoroacetone.

11. The composition of claim 1 wherein the stabilizing agent is 3,5-disulfonylpyrocatechol.

70 12. A hydrazinium diperchlorate based propellant composition capable of curing to a solid and stabilized toward vibrational and thermal shock consisting of the following components in the proportions indicated.

(a) about 10 to 40 parts by weight of a combustible polymeric hydrocarbon fuel binder including a curing agent in admixture therewith.

- (b) about 45 to 85 parts by weight of hydrazinium diperchlorate,
- (c) about 0 to 25 parts by weight of propellant adjuvants,
- (d) about .85 to 8.5 parts by weight of a metal chelating agent.

13. A hydrazinium diperchlorate based propellant composition capable of curing to a solid and stabilized toward vibrational and thermal shock consisting of:

- (a) about 10 to 40 parts by weight of a combustible polymeric hydrocarbon fuel binder including a curing agent in admixture therewith,
- (b) about 45 to 85 parts by weight of hydrazinium diperchlorate,
- (c) about 0 to 25 parts by weight of propellant adjuvants,
- (d) about .85 to 8.5 parts by weight of a metal chelating agent selected from the group consisting of:

Alkylenediamines

Alkylenetriamines

Polycarboxylic acids

Nitrilotriacetic acid

Amino acids

Peptides

The acids and salts of alkylenediamines and alkyl-enetriamines

Hydroxy acids

Hydroxy aldehydes

$\beta$ -ketones

Phenolics.

14. The composition of claim 13 wherein

- (a) the combustible fuel binder is a carboxyl containing hydrocarbon resin, and
- (b) the metal chelating agent is ethylenediaminetetra-acetic acid.

15. The composition of claim 13 wherein

- (a) the combustible fuel binder is a carboxyl containing hydrocarbon resin, and
- (b) the metal chelating agent is sodium tripolyphosphate.

16. The composition of claim 13 wherein

- (a) the combustible fuel binder is a carboxyl containing hydrocarbon resin, and
- (b) the metal chelating agent is nitrilotriacetic acid.

17. The composition of claim 13 wherein

- (a) the combustible fuel binder is a carboxyl containing hydrocarbon resin, and
- (b) the metal chelating agent is methionine.

#### References Cited

##### UNITED STATES PATENTS

|           |         |                     |        |
|-----------|---------|---------------------|--------|
| 3,006,743 | 10/1961 | Fox et al. -----    | 149—36 |
| 3,130,096 | 4/1964  | Pruitt et al. ----- | 149—19 |
| 3,155,552 | 11/1964 | Vriesen -----       | 149—19 |

25 BENJAMIN R. PADGETT, Primary Examiner

U.S. Cl. X.R.

149—20, 36